

H. R. WARDELL,  
BITUMINOUS STRUCTURAL MATERIAL,  
APPLICATION FILED JULY 24, 1908.

958,450.

Patented May 17, 1910.

FIG. I.



FIG. II.



WITNESSES:

John C. Bergner.  
Wm. K. Perl.

INVENTOR:

HENRY ROBBINS WARDELL,  
by his Attorneys  
Macy & Page

# UNITED STATES PATENT OFFICE.

HENRY ROBBINS WARDELL, OF PHILADELPHIA, PENNSYLVANIA.

## BITUMINOUS STRUCTURAL MATERIAL.

958,450.

Specification of Letters Patent. Patented May 17, 1910.

Application filed July 24, 1908. Serial No. 445,083.

To all whom it may concern:

Be it known that I, HENRY ROBBINS WARDELL, of Philadelphia, in the county of Philadelphia and State of Pennsylvania, have invented certain new and useful Improvements in Bituminous Structural Materials, of which the following is a specification, reference being had to the accompanying drawings.

My improvements relate to a structural material in the form of a composite sheet composed of bituminous cements combined with textile or felted fabrics, and it is the object of my invention to produce such a composite sheet having sufficient strength and rigidity to be in itself a self-supporting structural material, as for example, for a wall or a roof of a building.

To this end my material is composed of several layers, of which the external or surface ones are essentially protective layers, while the internal layer is a stiffening one, having both strength and rigidity so that, especially when corrugated, it may be used by itself to form the roof or the wall of a building.

Many composite roofing sheets or other forms of sheathing sheets have been made by the combination of felted and textile materials with bituminous cements, but it has always heretofore been supposed that such bituminous cements were too soft, especially when exposed to higher sun temperatures, to admit of their attaining a permanent consistency which would make the sheet rigid enough without brittleness to be useful as a structural material in itself. Consequently, all these previous bituminous composite sheets have been applied to an al-

ready existing surface, usually of boards, and have served only as sheathing therefor, but the sheet which I have invented possesses such strength and rigidity without brittleness that it may be corrugated and will retain its corrugation even under the extreme heat of the summer sun. In contradistinction to these sheathing sheets my invention is capable of being applied just as metallic structural sheets are now applied for the purpose of making the walls or roof of other parts of a building, without other sustaining means than the ordinary wooden or metal framework used in such cases.

My invention depends upon the principle, discovered by myself, that by employing external protective layers, an internal bitu-

minous sheet may be made and maintained with such consistency, rigidity and strength as to successfully hold its shape against the ordinary distorting strains to which such structural materials are subject, notwithstanding the deteriorating influences of the atmosphere, weather and sun. It is obvious that such a sheet is of very great value in that it enables buildings to be constructed more cheaply, dispensing entirely with the material ordinarily used for the walls or roofs, since possessing as it does water-proof, weather-proof, and fire resisting qualities, the sheet serves in itself to form a lasting wall or roof without the use of any other material than the supporting framework. Being unaffected by moisture or the corrosive gases which attack iron, it is a more durable substitute for corrugated iron sheets as a structural material.

In United States Letters Patent No. 851,331, granted to me under date of April 23rd, 1907, for a compound roofing sheet, I have described a composite bituminous sheet having certain of the characteristics of my present invention, and like it in some of its parts. But the roofing sheet thus previously patented by me did not possess the strength and rigidity requisite to allow the sheet to be corrugated or to hold its shape. Consequently, such sheet required a supporting surface for its application. It was, therefore, quite a different thing from my present invention, but in so far as certain of the parts of my present invention correspond to similar parts in the sheet previously patented, I may refer to my previous patent for the description of such parts without here repeating it.

In the accompanying drawing, Figure I, represents a portion of a composite corrugated sheet embodying my invention. Fig. II, illustrates my invention as applied to a corrugated sheet of different construction.

Primarily my present structural material is a composite sheet built up of two kinds of layers. But each of these layers may itself be composite so that the entire sheet may contain a large number of layers, but for functional distinction it is convenient to sub-divide all the layers into two, to wit: a rigid strengthening and sustaining layer, and an external protective layer.

Referring to Fig. I, of the drawing, it will be observed that the material is shown with its layers successively cut away so as to

disclose the structure as it is built up by the superimposition of successive layers. Of these, 1 is an external protective layer, 2, is the central strengthening layer, and 3, another protective layer. The external layers 1, and 3, consist of a felted fabric or other similar basis, such as roofing paper, or roofing felt, or wool felt, thoroughly saturated by an asphaltic or bituminous compound as 10 described in my previous patent, to which reference is made for description of the protective layers. Upon the surfaces of this saturated protective layer additional thin layers of bituminous material may be applied, these being so thin as not to be capable 15 of disclosure in the drawing. It is upon the central layer 2, that my present invention depends. This is preferably formed of a hard pure native bitumen, such as grahamite, wurtzilite, gilsonite or the like. This is 20 properly fluxed until it is of such consistency at 77° Fahrenheit, that when tested for five seconds with a No. 2 cambric needle under a hundred gram weight, it will be 25 penetrated to a depth of 0.10 mm. It is obvious that the consistency of this cement may be slightly varied, depending upon the viscosity of the native bitumen employed, so long as the main object is attained, which is 30 to produce a piece of structural material which will retain its shape and corrugation under maximum sun temperatures. To some extent the climatic conditions under which the structure is to be used will influence the 35 consistency of this cement, for obviously a harder material must be employed in the tropics than in colder regions. To increase the strength of this layer I prefer to embed therein a layer of coarse burlap or wire 40 mesh 5. The wire mesh to be employed may vary from say a twelve wire mesh to a three-eighths mesh wire. I prefer the wire mesh to the burlap, since it has greater strength and some rigidity, but for cheap 45 forms of construction the burlap may be employed. The thickness of this central layer may vary according to the strength required. I have found that a thickness of about 1/16 of an inch is sufficient for ordinary purposes. 50 To each side of the central layer 2, thus formed, protective layers 1, and 3, are applied, the three being united in the course of their manufacture to form one substantially integral structure. It is obvious that 55 if desired for increased strength the central layer may be reduplicated, or increased in size.

In Fig. II, I have shown an embodiment of my invention in which the strength and 60 rigidity of the material is increased, by additional layers of heavy Manila paper 4, 4, interposed on either side of the central layer between it and the external protective layers, and these layers of Manila paper

may be repeated to whatever extent is found 65 desirable. After the composite sheet comprising my invention has been thus built up, it is, while still soft from the heat of manufacture, corrugated by the use of ordinary corrugating rolls, or other suitable means, 70 and by reason of the hard consistency of the central layer, the corrugations thus imparted are retained, so that the entire sheet has structural or self-sustaining properties 75 similar to those of the ordinary corrugated metallic roofing sheet. When tested at ordinary temperatures the corrugated sheet may be walked upon by a heavy person without appreciable distortion of the corrugations. Accordingly the sheets thus prepared are employed as has been explained 80 to form the wall or the roof or other structural part of the building without other sustaining surfaces. It is thus distinguished from roofing sheets, not only in its self- 85 sustaining capacity, but by its method of application. Roofing sheets are nailed to a wooden backing and the joints are rendered tight and waterproof by a bituminous varnish or liquid cement. My structural sheets 90 may be used in the same manner as corrugated iron attached only to a frame and with overlapping joints without cementing. It will be understood that it would be difficult if not impossible, to secure to this central sheet the requisite strength and self- 95 sustaining qualities, and at the same time to maintain them under atmospheric deteriorating influences, were it not for the external protecting sheet which shields the 100 strengthening sheet from such influences, so that the bituminous material although hard, may possess and maintain sufficient life, (due in the main to the manner in which the bitumen has been fluxed), to prevent 105 its becoming brittle and breakable under the influences of sun and air and weather. The external protective sheets effectually retain the vitality and strength of the central layer for a long time under all ordinary 110 conditions of usage.

Having thus described my invention I claim:

A composite corrugated structural sheet comprising a strong rigid layer of hard 115 bituminous material reinforced by a vegetable or metal textile embedded therein, and having sufficient consistency to retain its corrugations under sun temperatures, in combination with one or more external protective bituminous sheets of a softer character.

In testimony whereof, I have hereunto signed my name, at Philadelphia, Pennsylvania, this twenty-third day of July 1908.

HENRY ROBBINS WARDELL.

Witnesses:

JAMES H. BELL,  
E. L. FULLERTON.